# EUROPEAN PATENT APPLICATION

(11) **EP 2 876 207 A1**
(43) Date of publication of application: **27.05.2015**
(21) Application number: 13194313.6
(22) Date of filing: 25.11.2013
(51) Int. Cl.: D21H 25/06, D21H 17/07, D21H 17/20, D21H 17/21, D21H 17/33, D21H 17/34, D21H 17/35, D21H 17/46, D21H 17/52, D21H 17/53, D21H 17/70, B27N 3/00, B27N 3/04

(54) **DryPulp for cureformed paper**

(71) Applicant: CEPI aisbl, 1050 Brussels (BE)
(72) Inventor: The designation of the inventor has not yet been filed
(74) Representative: Kinkeldey, Daniela

(57) **Abstract**

The present invention relates to a process comprising a non-water sheet forming technology using high concentration of cellulose fibres suspended in a high viscosity liquid.

## Description

The present invention relates to a process comprising a non-water sheet forming technology using high concentration of cellulose fibres suspended in a high viscosity liquid.

### BACKGROUND OF THE INVENTION

Today's paper machines require huge amounts of water for a number of reasons: the fibres need to be held at low concentration to avoid flocculation and to allow pumping as well as to enable a smooth formation as well as sufficient paper strengths. Removing the water at later stages requires a lot of energy. Tomorrow's paper machines should operate with in principle no water, which would eliminate the need for drying, the most energy intensive part of papermaking. In order to achieve this goal, a radically new technology for manufacturing has to be developed.

The dominant feature of a suspension composed of wood fibres and water is its inherent propensity to form bundles of mechanically entangled fibres, i.e. fibre flocs[1]. This is a feature closely connected to the concentration of fibres in water [2,3], which lies between 0.5-3% since higher concentration are not technically possible.

However, one possibility to avoid the flocculation of fibres that gives a poor sheet structure is to dramatically increase the viscosity of the fluid where the fibres are dispersed[2]. But, if only viscosity is increased dramatically the forces on the fibre surfaces levels will disintegrate the fibres[4]. If this detrimental effect can be avoided, it will allow forming at high concentration.

### SUMMARY OF THE INVENTION

It is one object of the invention provide a new process, which overcomes the above outlined problems.

The present invention therefore provides a process for producing paper comprising
a step (i) of treating fibres to protect them from shear,
a step (ii) of suspending the fibres after step (i) in a viscous solvent to obtain a suspension,
a step (iii) of forming a sheet with the suspension after step (ii),
a step (iv) of removing solvent of the sheet after step (iii), and
a step (v) of curing the sheet after step (iv) by curing.

By this process, paper will be made by applying an innovative non-water sheet forming technology using high concentration of cellulose fibres suspended in a high viscosity liquid. The biggest energy saving impact may result from eliminating not only the drying section, but also the needs for refining, vacuums in the process and huge flows in the white water recirculation. This would mean 28% energy saving and 61% CO₂ saving. This process enables single or multi-layer structure, thus opening new opportunities for functionalization of paper as well as with significantly reduced capital investments.

### DETAILED DESCRIPTION OF THE INVENTION

Before the present invention is described in detail below, it is to be understood that this invention is not limited to the particular methodology, protocols and reagents described herein as these may vary. It is also to be understood that the terminology used herein is for the purpose of describing particular embodiments only, and is not intended to limit the scope of the present invention which will be limited only by the appended claims. Unless defined otherwise, all technical and scientific terms used herein have the same meanings as commonly understood by one of ordinary skill in the art.

Throughout this specification and the claims which follow, unless the context requires otherwise, the word "comprise", and variations such as "comprises" and "comprising", will be understood to imply the inclusion of a stated integer or step or group of integers or steps but not the exclusion of any other integer or step or group of integers or steps. In the following passages different aspects of the invention are defined in more detail. Each aspect so defined may be combined with any other aspect or aspects unless clearly indicated to the contrary. In particular, any feature indicated as being preferred or advantageous may be combined with any other feature or features indicated as being preferred or advantageous.

The term "resin" as used herein relates to any liquid, solid, semisolid or viscous substances of plant origin, such as copal, rosin, and amber, used principally in lacquers, varnishes, inks, adhesives, synthetic plastics, and pharmaceuticals and any physically similar synthetics, or chemically modified natural resins including thermoplastic materials such as polyvinyl, polystyrene, and polyethylene and thermosetting materials such as polyesters, epoxies, and silicones that may be used with fillers, stabilizers, pigments, and other components to form plastics.

As used herein, a "viscous solvent" is a solvent having a dynamic viscosity of 0.01 to 1 kg/ms (Pa. s) measured with a viscometer at 20 °C.

Some documents are cited throughout the text of this specification. Each of the documents cited herein (including all patents, patent applications, scientific publications, manufacturer's specifications, instructions, DIN norms etc.), whether supra or infra, are hereby incorporated by reference in their entirety. Nothing herein is to be construed as an admission that the invention is not entitled to antedate such disclosure by virtue of prior invention.

As mentioned, the invention provides a process for producing paper comprising
a step (i) of treating fibres to protect them from shear,
a step (ii) of suspending the fibres after step (i) in a viscous solvent to obtain a suspension,
a step (iii) of forming a sheet with the suspension after step (ii),
a step (iv) of removing solvent of the sheet after step (iii), and
a step (v) of curing the sheet after step (iv) by curing.

In particular, the invention provides a process for producing paper comprising
a first process of preparing a suspension of fibres in a high viscosity solvent, wherein the suspended fibres have been modified to be protect from shear, and
a second process of cureforming.

In particular, in step (i) a "shear reduction layer" or a drag-reducing (lubricating) layer is implemented to protect the fibres from shear. This may be done by creating a low viscosity layer surrounding the fibre suspended in a high viscosity liquid that will prevent flocculation and allow processing at high concentration.

The application relates to the use of two main technologies that are combined with the generic process of layered material structures:
1° Preparation of a suspension, the "DryPulp", having a high viscosity liquid/resin where the suspended fibres have been modified to have protective drag-reducing (lubricating) layers at the fibre surface.
2° Forming via a forming/casting process, i.e. "CureForming", using the generic concept of layering for functionalised papermaking.

DryPulp technology

The first technology starts with dry (preferably <10% water content) fibres. Accordingly, the fibres used in step (i) have a water content of 0 to 20 wt%, preferably 5 to 15 wt%, and more preferably 10 to 12 wt%. Moreover, the fibres used in step (i) may be obtained from recycled or from virgin pulp.

The fibres are mixed into a high viscosity liquid, i.e. a resin, at high fibre concentration (up to 40% of fibres). Specifically, the suspension obtained in step (ii) may have a fibre concentration of 10 and 45 wt.-%, preferably 20 to 40 wt.-% and more preferably 30 to 40 wt.-%.

The liquid/resin may be constituted of a bio-based polymer, oligomer or monomer, which can be cross-linked during the curing process in order to form a fixed structure. The resin should be seen as a generic technology platform. Similarly to the possibility to choose fibres raw material, the resin will be available in many variants targeted at different needs (bulk, opacity, moldability, printing, barrier properties ...) that all fulfils the base requirement for being able to be used to form a sheet structure at very high fibre concentrations without excessive flocculation and without detrimental effects on the fibres.

The fibres may be modified chemically such that they will give rise to the protective "shear reduction layer" closest to the fibre surface. The possibility of modifying the resin to allow processing (rheology modification) has been exploited for processing within other areas such as e.g. in paints with excessive concentration of pigments or in biomass extrusion[5]. The resin and the fibres thus form a compatible system, which is called "DryPulp".

In step (i) amino acids may be used to protect the fibres from shear. Specifically, one possible embodiment of this application is to use bio-based substances such as amino acids to functionalize the surface of the cellulosic fibre. These will modify the docking points and introduce bulky side chains that push the individual fibres apart. This will modify the viscosity of the medium in the proximity of the fibres.

### - CureForming technology

By using the second technology, the DryPulp will allow forming of a thin sheet without excessive flocculation due to the high viscosity of the resin. Hence a fibre network similar to paper that is made today can be formed with up to 40% fibre content. There are several methods of sheet forming and one possible embodiment is to use a technology combining continuous resin casting with today's forming technology. The DryPulp is formed as a sheet, containing up to 40% fibres. After forming the sheet solvent is removed. Preferably, in step (iv) the solvent is removed by pressing the sheet e.g. subjected the sheet to a pressing stage where resin is removed similarly to today's pressing operation where water is removed. Compared to water the resin is not bound within the fibres and can thus easily be removed by the pressing operation. Typically, after step (iv) the sheet has a fibre concentration of 50 and 90 wt.-%, preferably 60 to 85 wt.-% and more preferably 70 to 80 wt.-%. Moreover, after the pressing operation the web may contain up to 80% fibres.

In step (v) the curing may be carried out by chemical additives, ultraviolet radiation, electron beam, heat or any combination thereof. The curing may cause cross-linking within the resin as well as between resin and the cellulose fibres. Curing can be made in several steps affecting different properties such as the resin only or the resin-protective layer interface. The resin-protective layer-fibre system will allow reversal of the curing, which will allow recycling of the resin as well as of the fibres.

To generate a controlled amount of bulk and thus stiffness depending of the product requirements to the formed sheet, the use of air or other gases as expanding elements within the sheet may be applied. This could be achieved either by having micro-capsules of air and gas within the resin that are activated during treatment in the pressing (crushed) or through substances that generates gas bubbles under the influence of the curing process or some other external forcing. One possibility is to use Sodium Bicarbonate to form gas bubbles[6]. This activation will generate carbon dioxide and the sheet will expand generating a bulky material. This is already used in speciality paper grades where an active energy beam is irradiated onto a foamable composition containing an acid generating agent and Sodium Bicarbonate. The irradiating energy generates an acid that activates the Sodium Bicarbonate that, in turn, generates the bubbles/foam.

### Layered structure and functionalization

Moreover, the sheet may be formed as a layered product. Typically, the layered product is formed by first forming simultaneously, e.g. in one nozzle, or separately at least two layers and then bringing the layers together. This will allow optimization towards desired product properties as well as addition of new functionalities. As an example, if a smooth surface is required, the expansion can be limited to take place within the middle layer of a three layered sheet, i.e. coating will be achieved during the forming process. Micro-bubbles may also be used in the final sheet in order to achieve opacity, which would remove the need for fillers.

### Carbon emission reduction

This process for paper and board products will contribute to decarbonisation through the energy savings gained from the elimination of the excessive need for vacuum, the friction losses in pressing and the drying of the base paper as well as drying of coating layers. As an example, the drying process in paper making alone consumes about half of the energy and today has the largest CO₂ impact.

An estimate of the energy demand for the process is as follows:
Curing of resins using heat in e.g. filter manufacturing, are made at temperatures up to 200°C.
This means that all material needs to be brought to that temperature. Given that the starting point is room temperature this means that one ton of material has to be heated about 180°C.
Assuming that the DryPulp has a specific heat capacity about the same as cellulose this gives that about 75 kWh/t is needed, given by: Since the concentration in the forming process is significantly high, the amount of mass (fibres+resin) that has to be pumped is less compared to traditional papermaking. On the other hand the viscosity goes up and the effective reduction in energy consumption for the DryPulp handling (a.k.a the stock preparation and
forming) will only be 50%[1]. The total energy demand for the complete "paper machine",
including drives, winding etc. will be 200 kWh/t. In addition, the energy demand for recycling will be reduced by 50%, coating will not be necessary since the product is coated in the forming process, and the absence of water removes energy costs for effluent treatment. Based on this, the technology will have an estimated total energy demand of 330 kWh/t. Looking at manufacturing of all paper and packaging grades (excluding sanitary and household), the energy demand of the papermaking process (excluding pulp production), is about 1550 kWh/t on average. Since the new process inly requires 330 kWh/t, as indicated above, this results in a reduction in energy demand by 79%. If the whole sector is considered, including pulp production as well as sanitary and household grades, this translates to a reduction in energy demand of 28%. Similarly, the process will cause 66 kg CO₂/t emissions compared to todays 370 kg/t for the manufacturing of paper and packaging grades (excluding pulp production and the sanitary and household grades), giving a reduction of 82%. For the whole sector this means a reduction by 61%.

Various modifications and variations of the invention will be apparent to those skilled in the art without departing from the scope of the invention. Although the invention has been described in connection with specific preferred embodiments, it should be understood that the invention as claimed should not be unduly limited to such specific embodiments. Indeed, various modifications of the described modes for carrying out the invention which are obvious to those skilled in the relevant fields are intended to be covered by the present invention.

### REFERENCES

1 Mason, S.G. (1948) "The Flocculation of Cellulose Fibre Suspensions", Pulp Paper Mag. Can. 99-104.
2 Kerekes (2009) "Rheology of fibre suspensions in papermaking: An overview of recent research", Nordic Pulp and Paper Research Journal, vol 21, issue 5, 2006, 598-612.
3 Schmid, C.F., Klingenberg, D.J. (2000) "Mechanical Flocculation in Flowing Fiber Suspensions", Physical Review Letters, 84 (2), pp. 290-293.
4 Suzuki, K., Okumura, H., Kitagawa, K., Sato, S., Nakagaito, A.N. & Yano, H. (2013) "Development of continuous process enabling nanofibrillation of pulp and melt compounding", Cellulose, vol. 20, no. 1, pp. 201-210.
5 Scott, C.T., Samaniuk, J.R., Klingenberg, D.J. (2011) "Rheology and extrusion of high-solids biomass", Tappi Journal, 10 (5), pp. 47-53.
6 Patent WO2011001791 A1, "Wood Powder-Containing Resin Molded Product and Method for Producing the Same".

## Claims

1. A process for producing paper comprising
a step (i) of treating fibres to protect them from shear,
a step (ii) of suspending the fibres after step (i) in a viscous solvent to obtain a suspension,
a step (iii) of forming a sheet with the suspension after step (ii),
a step (iv) of removing solvent of the sheet after step (iii), and
a step (v) of curing the sheet after step (iv).

2. The process according to claim 1, wherein the fibres used in step (i) have a water content of 0 to 20 wt%, preferably 5 to 15 wt%, and more preferably 10 to 12 wt%.

3. The process according to claim 1 or 2, wherein the fibres used in step (i) are obtained from recycled or from virgin pulp.

4. The process according to any of the preceding claims, wherein the viscous solvent is selected from uncured resins, and is preferably selected from polymers, oligomers or monomers.

5. The process according to any of the preceding claims, wherein in step (i) amino acids are used to protect the fibres from shear.

6. The process according to any of the preceding claims, wherein the suspension obtained in step (ii) has a fibre concentration of 10 and 45 wt.-%, preferably 20 to 40 wt.-% and more preferably 30 to 40 wt.-%.

7. The process according to any of the preceding claims, wherein the sheet is formed as a layered product in step (iii).

8. The process according to claim 7, wherein the layered product is formed by first forming simultaneously or separately at least two layers and then bringing the layers together.

9. The process according to any of the preceding claims, wherein in step (iv) the solvent is removed by pressing the sheet.

10. The process according to any of the preceding claims, wherein after step (iv) the sheet has a fibre concentration of 50 and 90 wt.-%, preferably 60 to 85 wt.-% and more preferably 70 to 80 wt.-%.

11. The process according to any of the preceding claims, wherein in step (v) the curing is carried out by chemical additives, ultraviolet radiation, electron beam, heat, or any combination thereof.

12. The process according to any of the preceding claims comprising a further step of using air or other gases as expanding elements within the sheet.

13. The process according to claim 13, wherein the further step comprises introducing micro-capsules of air or the other gases within the viscous solvent.

14. The process according to claim 13, wherein the further step comprises introducing substances that generate gas bubbles under the influence of step (v) or other external forcing.
